

R. C. BENNER & H. F. FRENCH.  
ELECTRIC BATTERY.  
APPLICATION FILED JULY 13, 1916.

1,289,365.

Patented Dec. 31, 1918.



INVENTOR.  
R. C. BENNER  
H. F. FRENCH  
BY *Sam J. Adams*,  
ATTORNEY

# UNITED STATES PATENT OFFICE.

RAYMOND C. BENNER AND HARRY F. FRENCH, OF FREMONT, OHIO, ASSIGNEES, BY  
MESNE ASSIGNMENTS, TO NATIONAL CARBON COMPANY, INC., A CORPORATION OF  
NEW YORK.

## ELECTRIC BATTERY.

1,289,365.

Specification of Letters Patent. Patented Dec. 31, 1918.

Application filed July 13, 1916. Serial No. 109,050.

To all whom it may concern:

Be it known that we, RAYMOND C. BENNER and HARRY F. FRENCH, citizens of the United States, residing at Fremont, in the county of Sandusky and State of Ohio, have invented a certain new and useful Improvement in Electric Batteries, of which the following is a full, clear, and exact description.

10 This invention relates to electric batteries, and while the invention is not necessarily limited thereto, we find it of especial value in connection with copper oxid cells having an alkaline electrolyte. In this type of battery the positive electrode usually consists of zinc and the negative electrode of powdered copper oxid inclosed in a perforated container. In some cases the negative electrode consists of a block of molded copper 15 oxid, but the electro-chemical action is, however, the same.

The complete battery consists of a jar having an alkaline electrolyte, such as sodium hydroxid, with an appropriate cover 20 from which the two electrodes are suspended. It has been found that sulfur has a remarkable property of materially increasing the voltage of the copper oxid cell, and in addition, causing an increase in service life. A patent application covering this 25 discovery was filed November 30, 1915, by R. W. Erwin, Serial No. 64,342.

We have made an improvement in the invention disclosed in such application, 30 which will now be described in detail. In the perforated container type of alkaline cell, some difficulty has been experienced in shipping the negative element on account of the oxid sifting out through the perforations.

40 We have found that an admirable way to prevent this is by mixing powdered sulfur with the copper oxid and heating it up to the softening or melting point of the sulfur, the heating being preferably carried on with 45 the mixture inside the perforated container to be used in the battery. When cool, the sulfur binds the oxid particles together so that they cannot sift out through the perforations. By using this special means of 50 incorporating the sulfur in the negative element, we obtain the high voltage and long life incident to the use of sulfur, as described in the previously mentioned application.

While there is no certain temperature to which the sulfur must be heated, the temperature must not be much above the melting point of sulfur, for we have found that best results are obtained when the sulfur is heated just sufficiently to bind the copper oxid particles together, that is, to a temperature in the neighborhood of 125° C.

Various amounts of sulfur may be used in conjunction with copper oxid. With a constant volume of depolarizer, a beneficial electro-chemical effect extends over the range 65 from 0.25% or less sulfur to 40% or more.

At about .5%, the binding effect of the sulfur just begins to be of value and the service is particularly high. Above .5%, the binding value increase steadily with the 70 amount of sulfur, while the electro-chemical advantages remain about the same or decrease somewhat until they begin to rise toward a fairly definite maximum which occurs in the vicinity of 25% sulfur. The 75 statements concerning the electro-chemical advantages are based upon calculations of ampere hour and watt hour service to a cut-off voltage of 0.5 volt.

Our improvement is not restricted to the 80 perforated container type of cell, as oxid blocks can be made with sulfur binder, and inclosed in a metal frame or attached in any way to a conducting support. We prefer, however, the perforated container type, 85 as it is easier to ship and no difficulty is encountered by fragments of oxid dropping off during use.

Having described our invention, what we 90 claim is:—

1. In electric batteries, a negative element 95 consisting of copper oxid bound together by sulfur.

2. In electric batteries, a negative element consisting of a perforated receptacle containing copper oxid bound together by sulfur.

3. In electric batteries, an alkaline electrolyte and a negative element consisting 100 of copper oxid bound together by sulfur.

In testimony whereof, we hereunto affix our signatures.

RAYMOND C. BENNER.  
HARRY F. FRENCH.